

# UNITED STATES PATENT OFFICE.

CHARLES FAUL, OF ST. KILDA, AND HENRY LAVERS, OF SURREY HILLS, VICTORIA, AUSTRALIA, ASSIGNEES, BY MESNE ASSIGNMENTS, TO MINERALS SEPARATION NORTH AMERICAN CORPORATION.

## SEPARATION OF MIXED SULFID ORES.

1,257,990.

Specification of Letters Patent.

Patented Mar. 5, 1918.

No Drawing. Continuation of application Serial No. 14,015, filed March 12, 1915. This application filed June 26, 1916. Serial No. 105,916.

*To all whom it may concern:*

Be it known that we, CHARLES FAUL, a subject of the King of England, residing at Moola, St. Leonards avenue, St. Kilda, State 5 of Victoria, Commonwealth of Australia, and HENRY LAVERS, a subject of the King of England, residing at Canterbury Road, Surrey Hills, State of Victoria, Commonwealth of Australia, have invented certain new and 10 useful Improvements in the Separation of Mixed Sulfid Ores, of which the following is a specification.

This invention is for improvements in or relating to the separation of mixed sulfid 15 ores and it refers more particularly to flotation separation whereby a fractional or differential flotation of certain sulfids, such as zinc sulfid (blende) from other sulfids, such as lead sulfid (galena), is obtained. This 20 application is a continuation of our application filed March 12, 1915, Serial Number 14,015.

The present invention relates to certain 25 improvements in what is commonly known as froth flotation separation in which the ores are subjected to agitation or aeration or both in a liquid to which is added a small proportion of a mineral-frothing agent, whereby a froth of the metalliferous particles of the ore is produced which floats to the 30 surface of the liquid, whence it is removed; as is described for example in the prior United States Patents No. 835,120 of November 6, 1906, No. 962,678 of June 28, 1910, 35 and No. 1064723 of June 17, 1913.

We have discovered that differential or 40 preferential flotation is effected by carrying out the froth flotation process in the presence of a mercury material, such as metallic mercury or a compound of mercury, such as an amalgam or a mercury salt.

According to this invention, therefore, a 45 process for the concentration of mixed sulfid ores consists in submitting the ore to flotation separation with agitation or aeration or both in the presence of metallic mercury or a mercury compound to obtain a float concentrate relatively rich in certain sulfids, such as zinc sulfid and a residue relatively 50 rich in other sulfids, such as lead sulfid.

This invention is applicable to various 55 modifications of the agitation-froth process

of concentrating ores to effect a differential or preferential flotation of the zinc sulfids, such as that in which an alkaline medium or 55 circuit water is employed having a bichromate of an alkali metal in solution.

In adapting this invention to the agitation-froth process, the apparatus may be, for example, of the form described in the prior 60 Patent No. 979857 of December 27, 1910, or No. 1064209 of June 10, 1913, or No. 1084196, of January 13, 1914, and the mercury material, such for example as metallic mercury 65 or a mercury compound such as an amalgam or a mercury salt may be placed in the apparatus in any convenient form or may be introduced with the circuit liquor or the pulp.

It has not previously been realized that 70 mercury played any part in preferential or differential separation, and our discovery lies in the fact that with many ores the presence of metallic mercury or its equivalent is 75 essential to a good separation of zinc sulfid (blende) or lead sulfid (galena) or other sulfids, or both.

The following example illustrates one application of this invention. A quantity of a 80 mixed zinc lead sulfid ore assaying galena 9%, blende 45% and pyrites 30% was mixed with water to form a freely flowing pulp to which was added potassium bichromate amounting to 0.4% on the ore, and sodium silicate amounting to 0.2% on the ore. Cresol amounting to one-half pound per ton of 85 ore was then added, and the mixture, which was maintained at a temperature of 140° F., was violently agitated to beat in air. The separating vessel was built of wood and mercury was placed in it. A float concentrate assaying 4.7% lead, 51.5% zinc and 8.6% iron was obtained.

Other experiments have been performed 90 in which similar separations have been effected of the zinc sulfid (blende) from the lead sulfid (galena) in a circuit water containing other salts in solution, such for example as sodium carbonate or sodium carbonate and sodium hydrogen sulfid in which metallic mercury has been present in the 100 agitation vessel.

Similar results have been obtained by the use of compounds of mercury in the agitation vessel.

What we claim as our invention and desire to secure by Letters Patent is:—

1. A process for the concentration of a mixed sulfid ore which consists in submitting such an ore to flotation separation with aeration in the presence of a mercury material to obtain a float concentrate relatively rich in zinc sulfid and a residue relatively rich in lead sulfid. 15
- 10 2. A process for the concentration of a mixed sulfid ore which consists in submitting such an ore to flotation separation with aeration in a circuit to which is added a small proportion of a mineral-frothing agent and in the presence of a mercury material to obtain a float concentrate relatively rich in zinc sulfid and a residue relatively rich in lead sulfid. 50
- 15 3. A process for the concentration of a mixed sulfid ore which consists in submitting such an ore to flotation separation with aeration in the presence of metallic mercury to obtain a float concentrate relatively rich in zinc sulfid and a residue relatively rich in other sulfids. 55
- 20 4. A process for the concentration of a mixed sulfid ore which consists in submitting such an ore to flotation separation with aeration in a circuit to which is added a small proportion of a mineral-frothing agent and in the presence of metallic mercury to obtain a float concentrate relatively rich in zinc sulfid and a residue relatively rich in other sulfids. 60
- 25 5. A process for the concentration of a zinc-lead sulfid ore which consists in submitting such an ore to flotation separation with aeration in the presence of a mercury material to obtain a float concentrate relatively rich in zinc sulfid and a residue relatively rich in lead sulfid. 65
- 30 6. A process for the concentration of a zinc-lead sulfid ore which consists in submitting such an ore to flotation separation with aeration in a circuit to which is added a small proportion of cresol and in the presence of metallic mercury to obtain a float concentrate relatively rich in zinc sulfid and a residue relatively rich in lead sulfid. 70
- 35 7. A process for the concentration of a zinc-lead sulfid ore which consists in submitting such an ore to flotation separation with aeration in a circuit to which is added a small proportion of a bichromate of an alkali metal and in the presence of metallic mercury to obtain a float concentrate relatively rich in zinc sulfid and a residue relatively rich in lead sulfid. 75
- 40 8. A process for the concentration of a zinc-lead sulfid ore which consists in submitting such an ore to flotation separation with aeration in the presence of a mercury material to obtain a float concentrate relatively rich in zinc sulfid and a residue relatively rich in lead sulfid.

ting such an ore to flotation separation with aeration in a circuit to which is added a small proportion of a mineral-frothing agent and in the presence of a mercury material to obtain a float concentrate relatively rich in zinc sulfid and a residue relatively rich in lead sulfid. 15

7. A process for the concentration of a zinc-lead sulfid ore which consists in submitting such an ore to flotation separation with aeration in a circuit to which is added a small proportion of a mineral-frothing agent and in the presence of metallic mercury to obtain a float concentrate relatively rich in zinc sulfid and a residue relatively rich in lead sulfid. 50

8. A process for the concentration of a zinc-lead sulfid ore which consists in submitting such an ore to flotation separation with aeration in a circuit to which is added a small proportion of cresol and in the presence of metallic mercury to obtain a float concentrate relatively rich in zinc sulfid and a residue relatively rich in lead sulfid. 60

9. A process for the concentration of a zinc-lead sulfid ore which consists in submitting such an ore to flotation separation with aeration in a circuit to which is added a small proportion of cresol and a small proportion of a bichromate of an alkali metal and in the presence of metallic mercury to obtain a float concentrate relatively rich in zinc sulfid and a residue relatively rich in lead sulfid. 70

In testimony whereof we have signed our names to this specification in the presence of two subscribing witnesses.

CHARLES FAUL.  
HENRY LAVERS.

Witnesses:

CLEM A. HART,  
G. L. CULLEN.

Copies of this patent may be obtained for five cents each, by addressing the "Commissioner of Patents  
Washington, D. C."